

Patented July 28, 1925.

1,547,931

# UNITED STATES PATENT OFFICE.

PAUL RICHARD KUEHNRICH, OF SHEFFIELD, ENGLAND.

PRODUCTION OF INGOTS AND OTHER METAL CASTINGS.

No Drawing.

Application filed January 23, 1924. Serial No. 688,097.

To all whom it may concern:

Be it known that I, PAUL RICHARD KUEHNRICH, a subject of the King of England, residing at Sheffield, in Yorkshire, England, have invented certain new and useful Improvements in or Relating to the Production of Ingots and Other Metal Castings (for which I filed an application for patent in Great Britain, Serial No. 3,769, on the 8th February, 1923); and I do hereby declare that the following is a full, clear, and exact description of the same.

This invention relates to the production of ingots and other metal castings, particularly those of steel and alloy steels, its object being to provide an improved process of treating ingots and other castings whereby they are produced in a state of virginal or initial softness, free from internal stresses, without the application of any further supply of heat, the heat of casting alone being sufficient.

It is, of course, well known to delay the cooling of ingots and other castings. For example when ingots are rolled on their casting heat they are removed from the moulds to soaking pits where they are allowed to remain until their temperatures are equalized before being rolled, and in other cases it is sometimes the practice to place ingots in ashes to cool more or less slowly during the ensuing twelve or twenty-four hours. According to the present invention, however, an ingot or other steel casting is stripped from its mould and placed in a suitable container under conditions which ensure very slow cooling. It is an important and essential feature of the invention that the surface or skin of the ingot or casting shall still be at a higher temperature than the recalescence point or critical hardening temperature of the metal concerned when the conditions to ensure slow cooling are completed. Such conditions are conveniently and preferably provided by covering the ingot or casting with kieselguhr or other known suitable heat insulating powder.

It is preferred to strip the ingot or casting as soon as possible after a skin of sufficient strength has formed to prevent "bleeding", distortion or other damage. The latest period to which stripping may safely be delayed in order to carry out the invention is when the coolest part of the skin or sur-

face has reached a temperature of from about 100° C. to 200° C. above the recalescence point, depending upon the time taken in stripping and placing the ingot or casting in the container and surrounding it with heat insulating material or conditions.

A further essential feature of the invention is that the rate of cooling of the ingot or casting shall be so slow that a period of at least about 96 hours is required for the metal to cool to a temperature at which it is immune from any hardening effect due to an increase in the rate of cooling and that the slow cooling conditions shall be maintained for that period. By such means both hardening of the metal and the production of internal stresses are prevented. As an example quite small ingots of from fifty to one hundred pounds in weight are slowly cooled through about four days and the conditions are such that they do not become cold until about the end of this period. This is the preferred rate of cooling for all sizes of ingots or castings in carrying out the present invention, a less thickness of heat insulating material being required for the larger ingots, as their natural rate of cooling is slower.

Although the present invention may be applied in the manufacture of any steel ingot or casting which is desired in a soft state, it is particularly useful in the manufacture of high speed steels, nickel chromium steels, rustless steel, and other special steel alloys. High speed steel ingots or ingots of like nature subjected to a treatment according to the invention are, when cold, in a state of virginal softness and ingots or castings when made from any of the various alloys so treated may be readily machined. Such ingots or castings are also quite free from internal stresses, and without removing any part of the surface by machining, chipping, or grinding, produce when forged out into bars material remarkably free from surface defects which are usually very prevalent in high class alloy steels.

What I claim is:—

The method of producing an ingot or other metal casting in a state of virginal softness by stripping it from the mould whilst its surface or skin is still at a higher temperature than the recalescence point or critical hardening temperature of the metal.

concerned, immediately placing it in a container and surrounding it with heat insulating material of sufficient thickness to reduce the rate of cooling so that a period of at least about 96 hours is required for the ingot or casting to become cold, substantially as specified.

In testimony whereof I hereunto affix my signature.

PAUL RICHARD KUEHNRICH.

Witnesses:

ARTHUR H. GREENWOOD,  
HAWTHORN WRIGHT.